

# UNITED STATES PATENT OFFICE.

MATHIAS OVROM SEM, OF CHRISTIANIA, NORWAY, ASSIGNOR TO DET NORSKE  
AKTIESELSKAB FOR ELEKTROKEMISK INDUSTRI, OF CHRISTIANIA, NORWAY,  
A BUSINESS ENTITY OF CHRISTIANIA, NORWAY.

## PROCESS OF FREEING METALS FROM COPPER.

1,425,701.

Specification of Letters Patent. Patented Aug. 15, 1922.

No Drawing.

Application filed April 4, 1919. Serial No. 287,589.

To all whom it may concern:

Be it known that I, MATHIAS OVROM SEM, a subject of Norway, and a resident of Christiania, Kingdom of Norway, have invented 5 certain new and useful Improvements in Processes of Freeing Metals from Copper, of which the following is a specification.

This invention relates to the removal of copper from metals containing the same. 10 The object of the invention is a treatment of the metal whereby the copper may be entirely removed or such amounts left as may be desired.

Ores such as iron ores, nickel ores, etc., 15 frequently contain small amounts of copper which in many cases is found in the metal manufactured from such ores. Its presence is often objectionable. Thus in the case of iron, the presence of copper is not desirable; it renders the iron brittle and unsuitable for use as steel; and in the manufacture of iron care has been taken that the copper contents do not exceed a certain amount. The metallurgists are not in entire agreement 20 as to the amount of copper permissible; as a rule 0.5% Cu is considered a maximum. In many cases it is, however, impossible to keep the copper contents as low as desired and a special treatment of 25 such iron will therefore be necessary to remove the copper partly or totally. I have studied this problem and have discovered a method whereby the copper contents may be eliminated or reduced to the desired degree in a convenient manner and with great 30 economy.

I have found that when iron containing a small amount of copper in the molten condition is treated with sulphur or sulphides 35 such as iron sulphides, silicon sulphide or other sulphides, there will always be an equilibrium between Cu in the metal and Cu in the sulphides. If a sulphide containing no or very little Cu is added to a metal 40 comparatively rich in copper, the Cu will then move from the metal to the sulphides and, in this manner the copper contents of the metal may be brought down to any desired degree. If one treatment is not sufficient, the sulphides comparatively rich in 45 copper may be removed and replaced by a new batch of sulphides free from copper. This treatment may be repeated any number of times until the desired result is obtained.

50 My process possesses special advantages

when the metal to be treated contains silicon or other elements such as carbon, phosphorus, or boron, having the property of lowering the solubility of copper sulphides in the metal.

For example if the metal to be freed from copper consists of iron and nickel and also contains silicon and copper, the presence of silicon will prevent nickel from entering the sulphides with which the metal is treated. 60 Further I may in a simple manner raise or lower the contents of Ni in the metal by removing or adding silicon. If more silicon is present in the metal than corresponding to the following equilibria:



at the temperature in question, iron sulphide will decompose and form FeSiS and 75 SiS<sub>2</sub>. The FeSi will dissolve in the metal and the percentage of Ni will sink accordingly. If on the other hand less silicon is present in the metal than corresponding to above equilibria, that is if silicon is removed by oxidation or by other means, iron will leave the metal and enter into the sulphides, whereby the percentage of Ni in the metal is raised.

In the following specific example I have 80 illustrated my method using as the metal to be freed from Cu iron containing also Ni and Si. In order to carry out my invention I then proceed as follows:

About 500 kilograms of iron containing 90 17% Si, 22% Ni, 1.2% Cu and 0.4% S are brought into a furnace which may be of any suitable type commonly used in metallurgy, but I prefer to use an electric furnace. In this furnace the metal is mixed with 30 95 kilograms of iron sulphide containing approximately 64% Fe, 36% S and 0.2% Cu and heated to about 1450° C. At this temperature both the iron and the sulphide will be in a molten state and the desired 100 reaction will take place resulting in the formation of copper sulphide from the copper, and iron from the iron sulphide. I have found that about one hour's treatment at above mentioned temperature gives a satisfactory result. I then interrupt the heating process and remove the molten metal 105 and the molten sulphides separately.

This may be done by first tapping the metal and then the sulphides, or in any other 110

well known convenient manner. The iron sulphide now being comparatively rich in Cu may of course be treated in a separate process for the recovery of Cu.

- 5 It is to be understood that my process is not limited to above example which has been given for illustration purposes only. The process may be carried out in similar manner if other raw materials are used.
- 10 Thus instead of using iron sulphide for the removal of copper, for example silicon sulphide or pure sulphur or both may be employed. The sulphide to be used will of course be chosen so as to form a useful alloy from the base of the sulphide and the metal treated. If the metal in question is nickel it will therefore be advantageous to use nickel sulphide for the removal of copper or if ferronickel is desired as a final product, iron sulphide may be used. In above specific example I have heated to a temperature of about 1450° C. The temperature necessary will of course vary according to the raw materials used and will mainly be determined by the melting point of the raw material in question. In order to obtain a good result a temperature above said melting point will generally be required.

15 The foregoing detailed description has been given for clearness of understanding and no undue limitation should be deduced therefrom, but the appended claims should be construed as broadly as permissible in view of the prior art.

20 35 What I claim as new and desire to secure by Letters Patent of the United States is:

1. The process of freeing metals from copper which comprises heating a metal containing copper to above its melting point and subjecting it to the action of sulphur in the form of a sulphide of the said metal whereby copper sulphide is formed, and separating said sulphide from the metal.
2. The process of freeing metals from copper which comprises heating iron containing copper and also containing silicon to above its melting point and subjecting it to the action of sulphur, whereby copper sulphide is formed, and separating said sulphide from the metal.
3. The process of freeing metals from copper which comprises heating iron containing copper and also containing silicon to above its melting point and subjecting it to the action of sulphur in the form of a

sulphide, whereby copper sulphide is formed, and separating said sulphide from the metal.

4. The process of freeing metals from copper which comprises heating iron containing 60 copper and also containing silicon to above its melting point and subjecting it to the action of sulphur in the form of an iron sulphide, whereby copper sulphide is formed, and separating said sulphide from 65 the metal.

5. The process of freeing metals from copper which comprises heating iron containing copper and also containing silicon and nickel to above its melting point and subjecting it to the action of sulphur, whereby 70 copper sulphide is formed, and separating said sulphide from the metal.

6. The process of freeing metals from copper which comprises heating iron containing 75 copper and also containing silicon and nickel to above its melting point and subjecting it to the action of sulphur in the form of a sulphide, whereby copper sulphide is formed, and separating said sulphide 80 from the metal.

7. The process of freeing metals from copper which comprises heating iron containing copper and also containing silicon and nickel to above its melting point and 85 subjecting it to the action of sulphur in the form of an iron sulphide, whereby copper sulphide is formed, and separating said sulphide from the metal.

8. The process of freeing metals from copper which comprises heating iron containing 90 copper and also containing silicon to substantially 1450° C. together with an iron sulphide, said iron sulphide reacting with the metallic copper present resulting in the 95 formation of copper sulphide and metallic iron, and separating said sulphide from the metal.

9. The process of freeing metals from copper which comprises heating iron containing 100 copper and also containing silicon and nickel to substantially 1450° C. together with an iron sulphide, said iron sulphide reacting with the metallic copper present resulting in the formation of copper, 105 sulphide and metallic iron, and separating said sulphide from the metal.

Signed at Christiania, Norway, this 18th day of March 1919.

MATHIAS OVROM SEM.